

# UNITED STATES PATENT OFFICE.

ALBERT SCHLUMBERGER, OF PARIS, FRANCE.

## WHITE SAFETY-PAPER.

### SPECIFICATION forming part of Letters Patent No. 443,116, dated December 23, 1890.

Application filed August 21, 1889. Serial No. 321,521. (No specimens.) Patented in France April 4, 1888, No. 194,222; in Belgium July 10, 1888, No. 82,515; in Austria-Hungary October 13, 1888, No. 9,662, and in Spain March 4, 1889, No. 9,320.

To all whom it may concern:

Be it known that I, ALBERT SCHLUMBERGER, a citizen of the Republic of France, residing at Paris, France, have invented a new and useful Improvement in the Art of Making White Safety-Paper, (for which I have obtained patents in France April 4, 1888, No. 194,222; in Belgium July 10, 1888, No. 82,515; in Austria - Hungary October 13, 1888, No. 9,662, and in Spain March 4, 1889, No. 9,320,) of which the following is a specification.

This invention relates to the preparation of a white safety-paper, by means of which the records written thereon cannot be forged or altered by means of acid or chloride of lime without the production of blue or brown spots.

My invention consists, essentially, in a paper impregnated with several ingredients in the form of resin compounds of metallic salts—  
e.g., a resinated ferrous-oxide salt with a mixture of a resin compound of plumbic ferro-cyanide (or ferro-cyanide of tin) and a resin compound of ferro-cyanide of manganese.

To form a very sensitive safety-paper I also add to the above mixture a mixture of resin compound of molybdenum salt or of resin compound of cadmium oxide, to which is added a specially-prepared compound of resinated sulphide of zinc, the whole worked together into the paper-pulp with a little borax having an alkaline reaction. Ordinarily the addition of an iron salt to ferro-cyanide of potassium would color the paper-pulp blue, especially when at the completion of the manufacture

the resin soap is decomposed by means of alum, as is done in coloring paper. This color is prevented by the isolating property of the resin compound of metallic salts, which in this instance is of prime importance. In order to fix the zinc sulphide directly upon the fibers a portion of the paper-pulp used is stirred with a quantity of zinc sulphate, and is then mixed with resin soap and sodium sulphhydrate. All these resin compounds are introduced for the purpose of causing the different metallic precipitates in alkaline state to adhere readily to the fibers. Otherwise the non-resinated individual precipitates would

during the process of manufacture mostly disappear and a worthless safety-paper would be produced.

The proportions of the different salts which I regard as best for the preparation of fifty kilos of paper are as follows: To a mass of one hundred and fifty kilos of paper-pulp, bleached and cleaned in the usual manner and which contains fifty kilos of dried paper fiber, there are added, preferably during the sizing operation of the machinery, the following ingredients:

First. One hundred to one hundred and fifty grams sulphate of iron, which is dissolved in a small quantity of water and is mixed with a small excess of resin soap. The precipitate thus produced is reddish-brown, but being small in quantity it does not affect the color of the paper, especially after the same has passed through the ordinary bluing operation.

Second. Then a mixture of six hundred to seven hundred grams borax, nine hundred to one thousand grams potassic cyanide dissolved in twenty liters of water, mixed with so much resin soap as will cause one kilo of resin to be present in the above-named soap solution.

Third. After the paper mass has been thoroughly stirred with this resin compound a solution of four hundred to five hundred grams plumbic acetate or zinc chloride in ten liters of water is added.

Fourth. The stirring is then continued and the following mixture is added: (a) ten liters of water and eight hundred to one thousand grams ferro-cyanide of potassium mixed with (b) one thousand to one thousand two hundred grams manganic sulphate of chloride. The reaction arising at this stage of the process is expressed in the following equation:



The precipitated manganic ferro-cyanide, being then converted into a resin compound by means of a solution of sixty liters of resin

soap containing three kilos of resin, is added to the mass of the pulp. If a salt of molybdenum or cadmium is to be used, then in the former case about four hundred grams of 5 ammonium molybdenate are taken, decomposed by an equivalent quantity of lead acetate, and added to the above mass. The reaction thus arising is expressed in the following equation:



Cadmium salt, on the contrary, is added to the manganese solution, and in the proportion of four hundred to five hundred grams. Whenever a molybdenum or cadmium salt is 20 employed, resinated zinc sulphide is added, which becomes fixed upon the fiber, as above stated, so that at each acid reaction, in case of forgery or alteration, a brown or dark colored molybdenum or cadmium sulphide is 25 formed upon the paper.

The proportion of zinc sulphide added to the above mass, in connection with the molybdenum or cadmium salts, is preferably two hundred and fifty grams for the above proportion of the ingredients.

Finally, and to complete the paper, the excess of resin soap which is not combined with the above-named metallic salts is decomposed by means of from three to four kilos of alum, as is usual in practice for sizing, except, when the mass shows too acid a reaction, it is neutralized by means of five hundred grams of borax or sodic phosphate, the purpose of this 35 addition being to fix the excess of alum in the form of a neutral precipitate.

The following formulas and equations express the principal reactions arising in the production of my safety-paper and when the same is acted on by acids or bleaching-powder 40 (hypochlorite of lime) for the purpose of effacing or altering any inscription thereon:



The addition of borax and an excess of 55 resin soap have for object only to keep the mixture alkaline, so as to prevent the formation of blue before the application of the acids, &c., for the purposes of alteration, as stated. When any of these acids—such as muriatic or 60 oxalic acid—are employed there occurs a displacement of the resin soap from the iron compounds fixed into the paper and the ensuing acidulation gives rise to blue stains, due

to the contact of the iron compounds and the prussiates or ferro-cyanides.

65

Example:



When hypochlorite of lime (bleaching-powder) is used, a brown stain, due to oxide of manganese, results, thus—



Under the addition of a molybdenum salts, the reaction exemplified in the following equation occurs in the pulp:



It is understood, of course, that the entire mixture comprising the ferrated paper-pulp is in an alkaline state. (Resin soap and borax in excess.) Acid acting on the paper so prepared and containing sulphide of zinc forms: 90  $\text{Mo}_3\text{S} + \text{PbS}$  (sulphide of molybdenum and sulphide of lead) as a brown sulphide stain. At the same time the acid acting on the ferro-cyanic acid evolved from the prussiate of lead and of manganese yields a blue stain with 95 the iron oxide in the paper.

Bleaching-powder produces brown stains, due to oxide of manganese, as already explained in connection with the first process.

Having thus described my invention, what 100 I claim, and desire to secure by Letters Patent, is—

1. A white safety-paper impregnated with resinated ferrous salt, a resin compound of plumbic ferro-cyanide, and a resin compound 105 of ferro-cyanide of manganese, substantially as and for the purposes set forth.

2. A white safety-paper impregnated with a mixture of resin compounds of metallic salts, in combination with a molybdenum salt 110 and a resin compound of zinc sulphide, substantially as and for the purposes set forth.

3. A white safety-paper impregnated with a resinated ferrous salt, a resin compound of plumbic ferro-cyanide, and a resin compound 115 of ferro-cyanide of manganese, in combination with a salt of molybdenum and a resin compound of zinc sulphide, substantially as and for the purposes set forth.

In testimony whereof I have signed my 120 name to this specification in the presence of two subscribing witnesses.

ALBERT SCHLUMBERGER.

Witnesses:

R. J. PRESTON,  
DAVID T. S. FULLER.